

W. R. SWAN.

PROCESS FOR THE TREATMENT OF IRON AND STEEL TO FORM A PERMANENT BLACK  
FINISH THEREON.

APPLICATION FILED JULY 30, 1913.

1,079,453.

Patented Nov. 25, 1913.



William R. Swan  
Inventor

Witnesses  
Harry B. Rook.  
T. M. Jones

By

N. S. Hise

Attorney

UNITED STATES PATENT OFFICE.

WILLIAM R. SWAN, OF BRIDGEPORT, CONNECTICUT.

**PROCESS FOR THE TREATMENT OF IRON AND STEEL TO FORM A PERMANENT BLACK FINISH THEREON.**

**1,079,453.**

**Specification of Letters Patent. Patented Nov. 25, 1913.**

Application filed July 30, 1913. Serial No. 782,078.

*To all whom it may concern:*

Be it known that I, WILLIAM R. SWAN, citizen of the United States, residing at Bridgeport, in the county of Fairfield and State of Connecticut, have invented certain new and useful Improvements in Processes for the Treatment of Iron and Steel to Form a Permanent Black Finish Thereon, of which the following is a specification.

10 The present invention relates to a new and novel process for the treatment of such metals as iron and steel to form a permanent black finish thereon, the said black finish being rust resisting under various atmospheric conditions and the ordinary conditions of use.

The object of the invention is to provide a process of this character which produces a durable and inexpensive finish upon the metal, which does not require numerous and repeated treatments of the metal, and which only requires a few minutes of time, whereas those processes now in common use require from two to eight hours.

25 With this and other objects in view, the process consists in treating the metal by successive steps in a novel manner as will be hereinafter described.

80 One form of apparatus for carrying out the process is illustrated by the accompanying drawing in which the figure is a vertical sectional view through a muffle furnace and a super-heater.

35 The iron or steel articles upon which it is desired to produce the permanent black finish are first placed in a suitable chamber such as a muffle furnace, together with a quantity of copper sulfate, sal-ammoniac or aluminum chlorid, tannin and glucose.

40 aluminum chloride, tannin, and glucose.  
These chemicals may be placed in the furnace in any manner, as a mixture in a single tray, and any suitable proportion of the chemicals may be employed, although I have found by experiment that the chemicals can be advantageously used in an ordinary muffle furnace in the following proportions.  
45

|                |     |       |
|----------------|-----|-------|
| Copper sulfate | 5   | part, |
| Sal-ammoniac   | 1   | " ,   |
| Tannin         | 3/8 | " ,   |
| Glucose        | 1/8 | " ,   |

The iron or steel articles together with the chemicals which have been placed in the muffle furnace are heated to about  $1050^{\circ}$  Fahr. and superheated steam injected into

55 Fahr. and superheated steam injected into

the furnace for a period of about thirty minutes. The steam for this purpose may be drawn from an ordinary water steam boiler at about five pounds pressure and superheated in any conventional manner. 60 After the iron and steel articles have thus been heated in the muffle furnace and subjected to the action of superheated steam in the presence of the chemicals they are withdrawn from the furnace and permitted to cool, after which they are submerged in paraffin oil which has been heated to a temperature of about 150° Fahr. The articles which have thus been treated are permitted to dry by exposure to the air, and a dead black rust resisting coating is thereby provided. 65 The pores of the metal will be opened up as it expands under the action of the heat, and this dead black rust resisting coating will penetrate into the metal as far as this opening up of the pores will permit. 70 75

The copper sulfate is a metallic salt and apparently forms the base on the metal which resists the rust, the other chemicals producing the finish which with the warmed paraffin oil gives the dead black desired. Should a heavier coating be desired, this can be obtained by a repetition of the process, although this is ordinarily not necessary. 80

It is not absolutely necessary to use tannin as an ingredient of the compound, and the tannin may be entirely omitted, if desired, although it has been found that a somewhat better finish is obtained where this ingredient is used. 90

In the drawing, which illustrates a sectional view through a muffle furnace and super-heater adapted for use in carrying out the process, the numeral 1 designates the muffle furnace which may be of the conventional construction and is provided with the usual door 2 through which the iron or steel articles 3 to be treated are placed in the furnace and removed therefrom. Vents 4 are provided in the walls of the furnace 1, the said vents being shown in the present instance as located in the top of the furnace. A shelf 5 is provided at the back of the furnace for supporting a tray 6 in which the chemicals are placed. A suitable opening 7 is provided through which the tray 6 may be placed upon the shelf or removed therefrom from the back of the furnace, a suit-

- is injected into the furnace through a pipe 9 which leads from a coil 10 in a superheater 11, the said coil receiving steam from an ordinary water steam boiler (not shown).
- 5 An oil burner 12 or the like of any conventional construction may be utilized in connection with the superheater for heating the steam. The articles 3 to be treated are placed in the furnace through the door 2 10 in the usual manner and acted upon as has previously been described.

Having thus described the invention, what I claim as new and desire to secure by Letters Patent, is:—

- 15 1. The process for the treatment of iron and steel to form a dead black rust resisting finish which includes the following steps, heating the iron being treated, subjecting it to the action of superheated steam 20 in the presence of a metallic salt adapted to form a base thereon while still heated, cooling and submerging the iron in heated paraffin oil.
2. The process of treating iron or steel 25 to produce a dead black rust resisting finish thereon, which includes the following steps, heating the iron being treated, subjecting it to the action of superheated steam in the presence of a metallic salt adapted to 30 form a base thereon and other chemicals adapted to coöperate therewith to produce a finish, cooling the iron and submerging it in heated paraffin oil.
3. The process of treating iron and steel 35 to produce a dead black rust resisting finish thereon, which includes the following steps, heating the iron being treated, subjecting it to the action of superheated steam in the presence of copper sulfate while thus heated, 40 cooling the article and submerging it in heated paraffin oil.
4. The process of treating iron and steel 45 to produce a dead black rust resisting finish thereon, which includes the following steps, heating the iron being treated, subjecting it to the action of superheated steam in the presence of copper sulfate and sal-ammoniac while thus heated, cooling the article and submerging it in heated paraffin 50 oil.
5. The process of treating iron and steel to produce a dead black rust resisting finish thereon, which includes the following steps,

heating the iron being treated, subjecting it to the action of superheated steam in the presence of copper sulfate, sal-ammoniac, and glucose while thus heated, cooling the iron and submerging it in heated paraffin oil.

6. The process of treating iron and steel 60 to produce a dead black rust resisting finish thereon, which includes the following steps, heating the iron being treated, subjecting it to the action of superheated steam in the presence of copper sulfate, sal-ammoniac, 65 and glucose, cooling the iron and submerging it in heated paraffin oil, and finally drying and cooling the iron by exposure to the air.

7. The process of treating iron and steel 70 to produce a dead black rust resisting finish thereon, which consists in heating the iron to about 1050° Fahr., subjecting it to the action of superheated steam in the presence of copper sulfate, sal-ammoniac and glucose 75 while thus heated, cooling the article and submerging it in paraffin oil heated to about 150° Fahr., and finally cooling and drying the iron by exposure to the air.

8. The process of treating iron and steel 80 to produce a dead black rust resisting finish thereon, which includes the following steps, heating the iron being treated, subjecting it to the action of superheated steam in the presence of copper sulfate, sal-ammoniac, 85 tannin, and glucose, cooling the iron and submerging it in heated paraffin oil, and finally drying and cooling the iron by exposure to the air.

9. The process of treating iron and steel 90 to produce a dead black rust resisting finish thereon, which consists in heating the iron to about 1050° Fahr., subjecting it to the action of superheated steam in the presence of copper sulfate, sal-ammoniac, glucose and 95 tannin, while thus heated, cooling the article and submerging it in paraffin oil heated to about 150° Fahr., and finally cooling and drying the iron by exposure to the air.

In testimony whereof I affix my signature 100 in presence of two witnesses.

WILLIAM R. SWAN.

Witnesses:

F. E. MORGAN,  
F. P. MUNICH.